



US007279071B2

(12) **United States Patent**  
**Williams et al.**

(10) **Patent No.:** **US 7,279,071 B2**  
(b5) **Date of Patent:** **Oct. 9, 2007**

|                                                                                   |                 |         |                        |
|-----------------------------------------------------------------------------------|-----------------|---------|------------------------|
| (54) <b>PAPER ARTICLES EXHIBITING WATER RESISTANCE AND METHOD FOR MAKING SAME</b> | 5,342,649 A     | 8/1994  | Sarokin                |
|                                                                                   | 5,415,923 A     | 5/1995  | Sarokin et al.         |
|                                                                                   | 5,514,429 A     | 5/1996  | Kamihgaraguchi et al.  |
|                                                                                   | 5,681,851 A     | 10/1997 | Lee et al.             |
|                                                                                   | 5,709,976 A     | 1/1998  | Malhotra               |
|                                                                                   | 5,938,825 A     | 8/1999  | Gaglani et al.         |
|                                                                                   | 5,985,076 A     | 11/1999 | Misuda et al.          |
|                                                                                   | 6,022,816 A     | 2/2000  | Dewar                  |
|                                                                                   | 6,034,081 A     | 3/2000  | Whittemore et al.      |
|                                                                                   | 6,048,575 A     | 4/2000  | Altavilla              |
|                                                                                   | 6,087,457 A     | 7/2000  | Tsai                   |
|                                                                                   | 6,183,814 B1    | 2/2001  | Nangeroni et al.       |
|                                                                                   | 6,197,805 B1    | 3/2001  | Smith                  |
|                                                                                   | 6,210,767 B1    | 4/2001  | Knauf                  |
|                                                                                   | 6,221,798 B1    | 4/2001  | Mahale et al.          |
|                                                                                   | 6,241,994 B1    | 6/2001  | Lee et al.             |
|                                                                                   | 6,358,576 B1    | 3/2002  | Adur et al.            |
|                                                                                   | 6,379,497 B1    | 4/2002  | Sandstrom et al.       |
|                                                                                   | 6,951,962 B2 *  | 10/2005 | Bottorff ..... 564/509 |
|                                                                                   | 2002/0040088 A1 | 4/2002  | Buchholz et al.        |
|                                                                                   | 2002/0185239 A1 | 12/2002 | Kimpimaki et al.       |

(65) **Prior Publication Data**

US 2004/0221976 A1 Nov. 11, 2004

**Related U.S. Application Data**

- (63) Continuation of application No. 10/117,358, filed on Apr. 5, 2002, now Pat. No. 6,645,642.
- (60) Provisional application No. 60/283,677, filed on Apr. 12, 2001, provisional application No. 60/283,055, filed on Apr. 11, 2001, provisional application No. 60/283,066, filed on Apr. 11, 2001.
- (51) **Int. Cl.**  
**D21F 11/00** (2006.01)
- (52) **U.S. Cl.** ..... 162/135; 162/164.1; 162/164.6; 162/168.1; 162/172; 564/509
- (58) **Field of Classification Search** ..... 162/135, 162/164.1, 164.6, 168.1, 168.2, 172, 175; 564/509

See application file for complete search history.

(56) **References Cited**

## U.S. PATENT DOCUMENTS

|               |         |                    |
|---------------|---------|--------------------|
| 3,174,874 A   | 3/1965  | Gernot et al.      |
| 3,293,114 A   | 12/1966 | Kenaga et al.      |
| 3,533,908 A   | 10/1970 | Hoogsteen          |
| 3,556,934 A   | 1/1971  | Meyer              |
| 4,040,900 A   | 8/1977  | Mazzarella et al.  |
| 4,133,688 A * | 1/1979  | Sack ..... 430/536 |
| 4,179,546 A   | 12/1979 | Garner et al.      |
| 4,279,794 A   | 7/1981  | Dumas              |
| 4,444,847 A   | 4/1984  | Fujioka et al.     |
| 4,448,807 A   | 5/1984  | Serlin             |
| 4,483,889 A   | 11/1984 | Andersson          |
| 5,017,416 A   | 5/1991  | Imperial et al.    |
| 5,087,457 A   | 2/1992  | Bryant et al.      |
| 5,125,996 A   | 6/1992  | Campbell et al.    |
| 5,133,835 A   | 7/1992  | Goettmann et al.   |

## FOREIGN PATENT DOCUMENTS

|    |                |         |
|----|----------------|---------|
| DE | 142 217 A      | 1/1987  |
| EP | 0629741 A1     | 6/1994  |
| EP | 0666368 A3     | 7/1996  |
| GB | 786543         | 10/1955 |
| GB | 903416         | 11/1959 |
| GB | 1373788        | 10/1971 |
| GB | 1533434        | 3/1976  |
| JP | 06-329834 A2   | 11/1994 |
| JP | 10034791 A2    | 7/1996  |
| WO | WO 00/44983 A  | 8/2000  |
| WO | WO 01/94512 A1 | 5/2001  |
| WO | WO 02/084026 A | 10/2002 |
| WO | WO 02/085539 A | 10/2002 |

## OTHER PUBLICATIONS

“Technology Review Series Triclosan and Its Impurities,” by J. Menoutis, Ph.D, copyright 1998-2001 Quantex Laboratories (2 pgs.).

\* cited by examiner

Primary Examiner—Mark Halpern

(74) Attorney, Agent, or Firm—Thomas W Barnes, III; Richard C. Stewart, II

(57) **ABSTRACT**

This invention relates to a process for preparing sized paper and paperboard which incorporates in the paper and paperboard at the size press size a composition comprising one or more “hydrophobic polymers” wherein hydrophobic polymers, the amount of such polymers and the weight ratio of starch to such polymer in the composition are selected such that the paper and paper board exhibits a Cobb Value equal to or less than about 25 and to a sized paper or paperboard web formed by the process.

29 Claims, 2 Drawing Sheets

Fig. 1. Felt Side Cobb Size Test



Fig. 2. Wire Side Cobb Size Test



Fig. 3. Felt Side Contact Angle



Fig. 4. Wire Side Contact Angle



**PAPER ARTICLES EXHIBITING WATER  
RESISTANCE AND METHOD FOR MAKING  
SAME**

RELATED APPLICATIONS

This application is a continuation of application Ser. No. 10/117,358 filed Apr. 5, 2002, now U.S. Pat. No. 6,645,642, and claims benefit of provisional application 60/283,055 filed Apr. 11, 2001, and claims benefit of provisional application 60/283,677 filed Apr. 12, 2001, and claims benefit of provisional application 60/283,066 filed Apr. 11, 2001.

BACKGROUND

1. Field of the Invention

The invention relates to the papermaking art and, in particular, to the manufacture of paper and paperboard which exhibit improved water resistance properties. This invention also relates to articles of manufacture made from such products such as file folders, non-corrugated containers, and the like.

2. Background of the Invention

Heavy weight cellulosic paper and paperboard webs and products made from same such as file folders and paperboard file containers are often subject to liquid or water damage during routine handling and long term storage. If moisture or aqueous liquid are absorbed by the paper or paperboard materials, the materials may become soggy, warped and/or weakened thereby reducing their usefulness and potentially allowing the liquids to contact and damage documents which may be stored in containers made with the paper or paperboard materials.

Surface sizing, i.e., the addition of sizing agents to the surface of a paper sheet that has been at least partially dried, is widely practiced in the paper industry, particularly for printing grades to improved water holdout (sizing). The most widely used surface sizing agent is starch. However, starch sizing alone has not been effective in providing water resistance to paper and paperboard products.

Accordingly, there exists a need for improved cellulose-based products, and in particular relatively heavy weight paper and paperboard products, which exhibit improved resistance to water and to a process for the manufacture of such water resistant cellulose-based products.

SUMMARY OF THE INVENTION

One aspect of this invention relates to a process for preparing sized paper and paperboard which incorporates in the paper and paperboard at the size press size a composition comprising one or more "hydrophobic polymers" either alone or in combination with one or more starches wherein hydrophobic polymers, the amount of such polymers and the weight ratio of said polymers and said starches are selected such that the paper and paper board web exhibits a Cobb value equal to or less than about 25 as determined by the Cobb Test described herein below and preferably has a contact angle equal to or greater than about 128° as determined by the contact angle test described herein below.

Another aspect of this invention relates to the sized paper or paperboard web formed by the method of this invention. The sized paper or paperboard web of this invention and products made from such web exhibits one or more beneficial properties such as resistance to water as determined by the "Cobb Test" and preferably by the "Contact Angle Test".

The web and products of the invention more preferably exhibit acceptable writability and are reputable.

BRIEF DESCRIPTION OF THE DRAWINGS

5 The above and other aspects and advantages of the invention will now be further described in conjunction with the accompanying drawings in which:

10 FIG. 1 is a graph of Cobb Value versus the amount of hydrophobic material picked up by the felt side of the paper.

15 FIG. 2 is a graph of Cobb Value versus the amount of hydrophobic material picked up by the wire side of the paper.

20 FIG. 3 is a graph of Contact Angle versus the amount of hydrophobic material picked up by the felt side of the paper.

25 FIG. 4 is a graph of Contact Angle versus the amount of hydrophobic material picked up by the wire side of the paper.

DETAILED DESCRIPTION OF THE  
INVENTION

In the process of this invention, a paper or paperboard web is treated at the size press with a sizing composition comprising at least one hydrophobic polymer in the absence of substantial absence of starch or in combination with one or more starches. The presence of the hydrophobic polymer in the size composition is critical for the advantages of this invention. As used herein, a "hydrophobic polymer" is a homopolymer, copolymer or terpolymer" selected from the group consisting of styrene acrylic emulsions (SAE), styrene acrylic Acid (SAA), styrene maleic anhydride (SMA), alkylated melamines wherein the alkyl moiety is branched or linear and has at least about 7 carbon atoms, paraffin wax, 30 polyurethanes, modified starch (hydrophobic starches), polyethylene, polymethylmethacrylate dispersion, alkyl ketene dimer, alkenyl ketene dimer, dispersed rosin and combination thereof. More preferred hydrophobic polymers are paraffin wax, alkylated melamines and most preferred 35 are alkylated melamines wherein the alkyl moiety is linear, more preferably where the alkyl moiety is linear and has at least 9 carbon atoms, and most preferably where the alkyl moiety is linear and has at least about 13 carbon atoms as for example a stearylated melamine, laurlated melamine, myristylated melamine, palmitated melamine and oleated melamine and a combination of paraffin wax and an alkylated melamine.

40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555

angle equal to or greater than about 133°. It is believed that these Cobb Values, and preferably the desired writability and contact angle values, can be obtained where the amount of hydrophobic polymer in the size composition is such that the amount of such polymer picked up by the paper and paper board is preferably at least about 0.4 wt %, more preferably at least about 0.5 wt % and most preferably at least about 0.9 wt % based on the total weight of the paper or paperboard, and in the embodiments of choice from about 1.3 to about 3.0 wt %.

The size composition may optionally include one or more starches. The amount of starch employed should not be such that the paper and paper board resulting from the process exhibits a Cobb Value equal to or less than about 25 and preferably exhibits a contact angle equal to or greater than about 128°. In the preferred embodiments of the invention, the amount of starch employed in the size composition is such that the weight ratio of starch to hydrophobic polymer picked up by the paper or paperboard is less than about 3 to about 1. In the more preferred embodiments of the invention, the amount of starch employed in the size composition is such that the weight ratio of starch to hydrophobic polymer picked up by the paper or paperboard is less than about 2 to about 1. In the most preferred embodiments of the invention, the amount of starch employed in the size composition is such that the weight ratio of starch to hydrophobic polymer picked up by the paper or paperboard is less than about 1 to about 1 and best if less than about 0.5 to about 1. In embodiments of choice, no or substantially no starch is employed in the size composition and no or substantially no starch is picked up by the paper or paperboard web.

The starch may be of any type, including but not limited to oxidized, ethylated, cationic and pearl, and is preferably used in aqueous solution. Illustrative of useful starches for the practice of this preferred embodiment of the invention are naturally occurring carbohydrates synthesized in corn, tapioca, potato and other plants by polymerization of dextrose units. All such starches and modified forms thereof such as starch acetates, starch esters, starch ethers, starch phosphates, starch xanthates, anionic starches, cationic starches and the like which can be derived by reacting the starch with a suitable chemical or enzymatic reagent can be used in the practice of this invention.

Useful starches may be prepared by known techniques or obtained from commercial sources. For example, the suitable starches include PG-280 from Penford Products, SLS-280 from St. Lawrence Starch, the cationic starch CatoSize 270 from National Starch and the hydroxypropyl No. 02382 from Poly Sciences, Inc.

Preferred starches for use in the practice of this invention are modified starches. More preferred starches are cationic modified or non-ionic starches such as CatoSize 270 and KoFilm 280 (all from National Starch) and chemically modified starches such as PG-280 ethylated starches and AP Pearl starches. More preferred starches for use in the practice of this invention are cationic starches and chemically modified starches.

In addition to the starch, small amounts of other additives may be present as well in the size composition. These include without limitation dispersants, fluorescent dyes, surfactants, deforming agents, preservatives, pigments, binders, pH control agents, coating releasing agents, optical brighteners, defoamers and the like.

Methods and apparatuses for treating a dried web of paper or paperboard with a sizing composition are well known in the paper and paperboard art. See for example "Handbook

For Pulp & Paper Technologies", 2<sup>nd</sup> Edition, G. A. Smook, Angus Wilde Publications (1992) and references cited therein. Any conventional size treatment method and apparatus can be used. Consequently, these methods and apparatuses will not be described herein in any great detail. By way of example, the size composition may be applied from a size press that can be any type of coating or spraying equipment, but most commonly is a puddle, gate roller or metered blade type of size press.

10 Any conventional paper or paperboard web can be used in the practice of this invention. Such webs and methods and apparatus for their manufacture are well known in the art. See for example *G. A. Smook* referenced above and references cited therein. For example, the paper and paperboard web can be made from pulp fibers derived from hardwood trees, softwood trees, or a combination of hardwood and softwood trees prepared for use in a papermaking furnish by any known suitable digestion, refining, and bleaching operations as for example known mechanical, thermomechanical, chemical and semichemical, etc., pulping and other well known pulping processes. In certain embodiments, at least a portion of the pulp fibers may be provided from non-woody herbaceous plants including, but not limited to, kenaf, hemp, jute, flax, sisal, or abaca although legal restrictions and other considerations may make the utilization of hemp and other fiber sources impractical or impossible. Either bleached or unbleached pulp fiber may be utilized in the process of this invention. Recycled pulp fibers are also suitable for use. In a preferred embodiment, the cellulosic fibers in the paper include from about 30% to about 100% by weight dry basis softwood fibers and from about 70% to about 0% by weight dry basis hardwood fibers. In the preferred embodiments of the invention, in addition to pulp fibers and optional additives, the paper or paperboard web also includes dispersed within the fibers and any other components expanded microspheres. Experimentation has shown that the combination of microspheres and hydrophobic polymer provides a paper or paperboard web and product made there from exhibiting even greater improvements in water resistance than the starch and hydrophobic polymer alone.

45 Expanded and expandable microspheres are well known in the art. See for example Expandable microspheres are described in co pending applications Ser. No. 09/770,340 filed Jan. 26, 2001 and Ser. No. 10/121,301, filed Apr. 11, 2002 and U.S. Pat. Nos. 3,556,934, 5,514,429, 5,125,996, 3,533,908, 3,293,114, 4,483,889, and 4,133,688; and UK Patent Application 2307487, the contents of which are incorporated by reference. All such microspheres can be used in the practice of this invention.

50 Suitable microspheres include synthetic resinous particles having a generally spherical liquid-containing center. The resinous particles may be made from methyl methacrylate, ethyl methacrylate, ortho-chlorostyrene, polyortho-chlorostyrene, polyvinylbenzyl chloride, acrylonitrile, 55 vinylidene chloride, para-tert-butyl styrene, vinyl acetate, butyl acrylate, styrene, methacrylic acid, vinylbenzyl chloride and combinations of two or more of the foregoing. Preferred resinous particles comprise a polymer containing from about 65 to about 90 percent by weight vinylidene chloride, preferably from about 65 to about 75 percent by weight vinylidene chloride, and from about 35 to about 10 percent by weight acrylonitrile, preferably from about 25 to about 35 percent by weight acrylonitrile.

60 The amount of microspheres may vary widely and depends on the desired expanded microsphere volume in the final paper product. Preferably the paper includes from about 0.5 to about 5.0 wt % expanded microspheres and more

preferably from about 1.0 to about 2.0 wt % by dry weight of the paper or paperboard web.

The web may also include other conventional additives such as, for example, starch, mineral fillers, sizing agents, retention aids, and strengthening polymers. Among the fillers that may be used are organic and inorganic pigments such as, by way of example, polymeric particles such as polystyrene latexes and polymethylmethacrylate, and minerals such as calcium carbonate, kaolin, and talc. Other conventional additives include, but are not restricted to, wet strength resins, internal sizes, dry strength resins, alum, fillers, pigments and dyes. For obtaining the highest levels of surface sizing in the processes of this invention, it is preferred that the sheet be internally sized, that is, that sizing agents be added to the pulp suspension before it is converted to a paper sheet. Internal sizing helps prevent the surface size from soaking into the sheet, thus allowing it to remain on the surface where it has maximum effectiveness. The internal sizing agents encompass any of those commonly used at the wet end of a fine paper machine. These include rosin sizes, ketene dimers and multimers, and alkenylsuccinic anhydrides. The internal sizes are generally used at levels of from about 0.05 wt. % to about 0.25 wt. % based on the weight of the dry paper sheet. Methods and materials utilized for internal sizing with rosin are discussed by E. Strazdins in *The Sizing of Paper*, Second Edition, edited by W. F. Reynolds, Tappi Press, 1989, pages 1-33. Suitable ketene dimers for internal sizing are disclosed in U.S. Pat. No. 4,279,794, which is incorporated by reference in its entirety, and in United Kingdom Patent Nos. 786,543; 903,416; 1,373,788 and 1,533,434, and in European Patent Application Publication No. 0666368 A3. Ketene dimers are commercially available, as Aquapel.RTM. and Precis.RTM. sizing agents from Hercules Incorporated, Wilmington, Del. Ketene multimers for use in internal sizes are described in: European Patent Application Publication No. 0629741 A1, corresponding to U.S. patent application Ser. No. 08/254, 813, filed Jun. 6, 1994; European Patent Application Publication No. 0666368 A3, corresponding to U.S. patent application Ser. No. 08/192,570, filed Feb. 7, 1994; and U.S. patent application Ser. No. 08/601,113, filed Feb. 16, 1996. Alkenylsuccinic anhydrides for internal sizing are disclosed in U.S. Pat. No. 4,040,900, which is incorporated herein by reference in its entirety, and by C. E. Farley and R. B. Wasser in *The Sizing of Paper*, Second Edition, edited by W. F. Reynolds, Tappi Press, 1989, pages 51-62. A variety of alkenylsuccinic anhydrides are commercially available from Albemarle Corporation, Baton Rouge, La.

The density, basis weight and caliper of the web of this invention may vary widely and conventional basis weights, densities and calipers may be employed depending on the paper-based product formed from the web. Paper or paperboard of invention preferably have a final caliper, after calendering of the paper, and any nipping or pressing such as may be associated with subsequent coating of from about 2 mils to about 30 mils although the caliper can be outside of this range if desired. More preferably the caliper is from about 4 mils to about 20 mils, and most preferably from about 7 mils to about 17 mils. Papers of the invention preferably exhibit basis weights of from about 17 lb/3000 ft<sup>2</sup> to about 300 lb/3000 ft<sup>2</sup>, although web basis weight can be outside of this range if desired. More preferably the basis weight is from about 30 lb/3000 ft<sup>2</sup> to about 200 lb/3000 ft<sup>2</sup>, and most preferably from about 35 lb/3000 ft<sup>2</sup> to about 150 lb/3000 ft<sup>2</sup>. The final density of the papers, that is, the basis weight divided by the caliper, is preferably from about 6 lb/3000 ft<sup>2</sup>/mil to about 14 lb/3000 ft<sup>2</sup>/mil although web

densities can be outside of this range if desired. More preferably the web density is from about 7 lb/3000 ft<sup>2</sup>/mil to about 13 lb/3000 ft<sup>2</sup>/mil and most preferably from about 9 lb/3000 ft<sup>2</sup>/mil to about 12 lb/3000 ft<sup>2</sup>/mil. Thus, in the 5 preferred embodiments of the invention the paper or paperboard has a relatively larger caliper in relation to its weight compared to conventional papers. In these preferred embodiments of the invention, the reduction in basis weight versus caliper is believed to be attributable at least in part to the large number of tiny voids in the paper associated with the expanded microspheres interspersed in the fibers with the microspheres causing, especially during the expansion process, a significant increase in the void volume in the material. In addition, the paper after drying operations is 10 calendered sufficient to achieve the final desired calipers discussed herein along with any desired surface conditioning of the web associated with the calendering operation. The impartation of a significantly increased void volume along with a relatively high caliper also has the effect of reducing 15 the density of the paper while retaining good stiffness and other properties important for use as stock for file folders and the like.

Preferably the process comprises: a) providing an aqueous pulp suspension; b) sheeting and drying the aqueous pulp suspension to obtain dried paper or paperboard web; c) treating the dried paper or paper or paperboard web by applying to at least one surface of the web a size composition containing one or more hydrophobic polymers and starch to form a treated paper or paperboard web; and d) 20 drying the paper to obtain sized paper or paperboard web.

In step a) of the preferred embodiment of this invention, an aqueous pulp suspension is provided. Methods of forming aqueous pulp suspensions are well known in the paper and paperboard art and will not be described in any great detail. See for example *G. A. Smook* referenced above and references cited therein. Any conventional aqueous pulp suspensions method can be used. The cellulosic fibrous component of the furnish is suitably of the chemically pulped variety, such as a bleached kraft pulp, although the invention is not believed to be limited to kraft pulps, and may also be used with good effect with other chemical pulps such as sulfite pulps, mechanical pulps such as ground wood pulps, and other pulp varieties and mixtures thereof such as chemical-mechanical and thermo-mechanical pulps.

While not essential to the invention, the pulp is preferably bleached to remove lignins and to achieve a desired pulp brightness according to one or more bleaching treatments known in the art including, for example, elemental chlorine-based bleaching sequences, chlorine dioxide-based bleaching sequences, chlorine-free bleaching sequences, elemental chlorine-free bleaching sequences, and combinations or variations of stages of any of the foregoing and other bleaching related sequences and stages. After bleaching is 35 completed and the pulp is washed and screened, it is generally subjected to one or more refining steps. Thereafter, the refined pulp is passed to a blend chest where it is mixed with various additives and fillers typically incorporated into a papermaking furnish as well as other pulps such as unbleached pulps and/or recycled or post-consumer pulps. The additives may include so-called "internal sizing" agents used primarily to increase the contact angle of polar liquids 40 contacting the surface of the paper such as alkenyl succinic anhydride (ASA), alkyl ketene dimer (AKD), and rosin sizes. Retention aids may also be added at this stage. Cationic retention aids are preferred; however, anionic aids 45 may also be employed in the furnish.

In addition, and prior to providing the furnish to the headbox of a papermaking machine, polymeric microspheres are preferably added to the pulp furnish mixture if desired as a component of the paper or paperboard web. The microspheres may be preexpanded or in substantially their final dimension prior to inclusion in the furnish mixture. The microspheres preferably are in the subsist in an "unexpanded" state in the original papermaking furnish from which the web is derived and, upon heating during the paper or paper board manufacturing process, undergo expansion in diameter such that in final sized paper paperboard web they are in an "expanded" state. It will be appreciated that this expansion has the effect of enabling an increased caliper and reduced density in the final paper product. It is also within the scope of the invention to include mixtures of expandable and already-expanded microspheres (or microspheres that are already substantially in their final dimensional state) in the papermaking furnish so that a portion of the microspheres will expand to a substantial degree in drying operations while the balance will remain in substantially the same overall dimensions during drying. The degree of expansion may vary widely. Preferably the degree of expansion is at least about 200% based on the volume of the unexpanded microspheres, more preferably at least about 300% and more preferably from about 300 to about 600% on the aforementioned basis. In their original unexpanded state, the center of the expandable microspheres may include a volatile fluid foaming agent to promote and maintain the desired volumetric expansion. Preferably, the agent is not a solvent for the polymer resin. A particularly preferred foaming agent is low molecular linear or branch alkane or alkene as for example isobutane, which may be present in an amount sufficient for the desired degree of expansion. In the preferred embodiments amount may range from about 10 to about 25 percent by weight of the total weight of the resinous particles. Suitable expandable microspheres can be prepared using known techniques or commercially as for example suitable microspheres are available from Akzo Nobel of Marietta, Ga. under the tradename EXPANCEL.

In step (b) of the process of this invention, the pulp suspension of step (a) is sheeted and dried to obtain dried paper or paperboard web. Methods and apparatuses for sheeting and drying a pulp suspension are well known in the paper and paperboard art. See for example *G. A. Smook* referenced above and references cited therein. Any conventional sheeting and drying method can be used. Consequently, these methods will not be described herein in any great detail. By way of example, the aqueous paper making stock furnish containing pulp, and other additives is deposited from the head box of a suitable paper making machine into a single or multi-ply web on a papermaking machine such as a Fourdrinier machine or any other suitable papermaking machine known in the art, as well as those which may become known in the future. For example, a so-called "slice" of furnish consisting of a relatively low consistency aqueous slurry of the pulp fibers along with the microspheres and various additives and fillers dispersed therein is ejected from a headbox onto a porous endless moving forming sheet or wire where the liquid is dewatered by gradually drained through small openings in the wire by vacuum in the forming section until a mat of pulp fibers and the other materials is formed on the wire. The dewatered wet mat or web is transferred from the forming section to the press section on specially constructed felts through a series of roll press nips that removes water and consolidates the wet web of paper. The web is then passed to an initial dryer section to remove most of the retained moisture and further

consolidate the fibers in the web. The heat of the drying section also promotes expansion of unexpanded microspheres that may be contained in the web.

In step (c) of the process of this invention, the dried paper or paper or paperboard web is treated by applying to at least one surface of the web a size composition comprising one or more hydrophobic polymers. Methods and apparatuses for treating a dried web of paper or paperboard with a sizing composition are well known in the paper and paperboard art. See for example, *G. A. Smook* referenced above and references cited therein. Other additives such as starch, pigments, and other additives may be applied to the web and incorporated therein by the action of the press if desired as described above in more detail.

In step (d) of the preferred embodiment of the process of this invention, the paper or paperboard web is dried after treatment with the size composition. Methods and apparatuses for drying paper or paperboard webs treated with a sizing composition are well known in the paper and paperboard art. See for example *G. A. Smook* referenced above and references cited therein. Any conventional drying method and apparatus can be used. Consequently, these methods and apparatuses will not be described herein in any great detail. After drying, the paper may be subjected to one or more post drying steps as for example those described in *G. A. Smook* referenced above and references cited therein. For example, the paper or paperboard web may be coated and/or calendered to achieve the desired final caliper as discussed above to improve the smoothness and other properties of the web. The calendering may be accomplished by steel-steel calendering at nip pressures sufficient to provide a desired caliper. It will be appreciated that the ultimate caliper of the paper ply will be largely determined by the selection of the nip pressure

An important property of the webs made according to the invention is their watershedability or resistance to wetting by aqueous fluids. Surface sized paper and paperboard webs produced by the process of this invention have water resistance properties that are substantially improved over those of paper and paperboard webs that is the same except that they have not been surface sized with a combination of starch and hydrophobic polymer in accordance with this invention. The resistance of the web to wetting by aqueous fluids can be determined by the Cobb Sizing Test, according to ASTM D-3285 (TAPPI T-441). Conventional, sized webs used for file folders have a five-minute water absorption in the range of from about 50 to 70 grams per square meter of paper tested. The web 10 containing holdout layer 12 and print receptive layer 14 preferably has a five minute water absorption in the range of from about 30 to about 40 grams per square meter. A tester for performing the Cobb sizing test consists of a hollow metal cylinder or ring (100, 25 or 10 cm<sup>2</sup> inside area). A metal base plate with a clamping device is used to hold the ring against the sample of paper to be tested and a neoprene mat. Neoprene gaskets may be used to seal the cylinder against the web when the test sample is uneven. An important component of the test apparatus is a solid stainless steel roller having a smooth face about 20 cm wide and weighing about 10 kg. Also used for the test is a 100 mL graduated cylinder, a balance with sensitivity of 0.01 grams or better, blotting paper, and a timer or stopwatch. A sample of paper or paperboard material to be tested is cut approximately 12.5×12.5 cm square from the coated web. The sample is weighed and placed on the neoprene mat. The cylinder is clamped upon the sample by locking a crossbar in place and tightening two knobs. If sample material is textured, a gasket is placed between the sample

and cylinder, carefully aligning the inner edges of each. The test liquid, in this case preferably water is poured into the test cylinder. The amount of test liquid is preferably 100 mL for 100 square centimeter cylinder. Proportionately less liquid is used for smaller cylinders. After pouring the liquid, the timer is started to provide a five-minute test. Longer and shorter test periods may be provided. At fifteen seconds before the expiration of the predetermined test period, the liquid is quickly poured from the cylinder, using care in not dropping any liquid on the untreated (outside) portion of the test specimen. The cylinder is removed from the sample and the sample is placed with wetted side up on a sheet of blotting paper. At exactly the end of the predetermined test period, a second sheet of blotting paper is placed on top of the sample to remove the surplus liquid by moving the hand roller once forward and once backward over the sample and blotting paper. Care should be taken not to exert downward force on the roller. The specimen is then folded after removing it from between the blotter sheets and re-weighed to the nearest 0.01 gram. The initial weight of the web is subtracted from the final weight of the sample and the gain in weight in grams is multiplied by 100 for a 100 cm<sup>2</sup> cylinder to obtain the weight of liquid absorbed in grams per square meter. The paper or paperboard of this invention exhibits a Cobb Value equal to or less than about 25, preferably equal to or less than about 23, more preferably equal to or less than about 21 and most preferably equal to or less than about 20.

In the preferred embodiments of the invention, the resistance of the web to wetting by aqueous fluids can also be determined by Contact Angle Test. Contact angle measurements are performed on narrow strips (1/4-1/3 inch) of paper cut diagonally across the sample. A water droplet (or other liquid) is deposited onto the surface of the paper. A video camera records the droplet over a period of ca. 4.5 sec. Frames are captured at 0.1 second intervals. Contact angles are then calculated using image analysis on the video images. The measurements are conducted at room temperature. Typically, six droplets are analyzed per sample. The instrument used is a First Ten Angstroms, FTA, Instrument. The contact angle is equal to or greater than about 128°, preferably equal to or less than about 130°, more preferably equal to or less than about 132° and most preferably equal to or less than about 133°.

The paper and paperboard web of this invention can be used in the manufacture of a wide range of paper-based

products where water resistance is desired using conventional techniques. For example, paper and paperboard webs formed according to the invention may be utilized in a variety of office or clerical applications. The web is preferably used for making file folders, manila folders, flap folders such as Bristol base paper, and other substantially inflexible paperboard webs for use in office environments, including, but not limited to paperboard containers for such folders, and the like. The manufacture of such folders from paper webs is well known to those in the paper converting arts and consists in general of cutting appropriately sized and shaped blanks from the paper web, typically by "reverse" die cutting, and then folding the blanks into the appropriate folder shape followed by stacking and packaging steps. The blanks may also be scored beforehand if desired to facilitate folding. The scoring, cutting, folding, stacking, and packaging operations are ordinarily carried out using automated machinery well-known to those of ordinary skill on a substantially continuous basis from rolls of the web material fed to the machinery from an unwind stand.

The following non-limiting examples illustrate various additional aspects of the invention. Unless otherwise indicated, temperatures are in degrees Celsius, percentages are by weight and the percent of any pulp additive or moisture is based on the oven-dry weight of the total amount of material.

#### EXAMPLE I

A series of paperboard samples at a basis weight of 124 lb/3000 ft<sup>2</sup> was prepared from a combination of 65% hard wood and 35% soft wood pulps. The paper was sized internally with ASA size and contained ground calcium carbonate as filler. The paper was dried before the size press to about 3% moisture. A size solution containing an ethylated starch, to which varying amounts of a hydrophobic polymer was added was used for application at the puddle size press on the paper machine and is driven into the sheet running through the size press nips. The pick-up of starch and additive were calculated using the starch: additive ratio and the amount of wet pickup measured at the size press during manufacture. The paperboard samples are described in more detail in Table I.

TABLE I

| Substrate | <sup>(1)</sup> Hydrophobic Polymer Pick-Up, wt % | <sup>(2)</sup> Starch Pick-Up, wt % | <sup>(3)</sup> Expandable Microspheres, wt % | Size Press Solids, wt % | Starch:Additive Ratio |
|-----------|--------------------------------------------------|-------------------------------------|----------------------------------------------|-------------------------|-----------------------|
| 1         | 0.00%                                            | 2.2%                                | 0%                                           | 11%                     | Starch only           |
| 2         | 0.21%                                            | 1.9%                                | 0%                                           | 11%                     | 9:1                   |
| 3         | 0.52%                                            | 1.6%                                | 0%                                           | 11%                     | 3:1                   |
| 4         | 0.88%                                            | 1.3%                                | 0%                                           | 11%                     | 1.5:1                 |
| 5         | 0.98%                                            | 1.0%                                | 0%                                           | 11%                     | 1:1                   |
| 6         | 1.35%                                            | 0.6%                                | 0%                                           | 11%                     | 0.42:1                |
| 7         | 1.27%                                            | 1.3%                                | 0%                                           | 15%                     | 1:1                   |
| 8         | n.d.                                             | 0.0%                                | 2%                                           | 11%                     | Starch Only           |
| 9         | 0.29%                                            | 2.6%                                | 2%                                           | 11%                     | 9:1                   |
| 10        | n.d.                                             | n.d.                                | 2%                                           | 11%                     | 3:1                   |
| 11        | n.d.                                             | n.d.                                | 2%                                           | 11%                     | 1.5:1                 |

TABLE I-continued

| Substrate | <sup>(1)</sup> Hydrophobic Polymer Pick-Up, wt % | <sup>(2)</sup> Starch Pick-Up, wt % | <sup>(3)</sup> Expandable Microspheres wt % | Size Press Solids, wt % | Starch:Additive Ratio |
|-----------|--------------------------------------------------|-------------------------------------|---------------------------------------------|-------------------------|-----------------------|
| 12        | n.d.                                             | n.d.                                | 2%                                          | 11%                     | 1:1                   |
| 13        | 1.58%                                            | 0.7%                                | 2%                                          | 11%                     | 0.42:1                |

The terms identified by superscripts are defined as follows:

<sup>(1)</sup>"Hydrophobic Polymer" is a stearylated melamine/paraffin wax obtained commercially from RohmNova under the tradename Sequapel ® 414.

<sup>(2)</sup>"Starch" is an ethylated starch obtained commercially from Penford under the tradename Penford 270.

<sup>(3)</sup>"Microspheres" is a expandable microsphere obtained commercially from Expance Inc. under the tradename "Expance".

15

## EXAMPLE II

The sample paperboards of Example I were evaluated to determine water resistance. The evaluation test used where the Cobb Test and the Contact, Angle Test described above. The samples were also evaluated subjectively using the following scale:

## (1) Excellent (A):

Water beads like water on a waxed surface and then when the paper is shaken off the water pretty much goes away. There could be some small remaining beads that need to be wiped off. There should also be no look of water penetrating the paper sheet over a 20 second period. A ballpoint pen or a pencil can write on the paper with minimal to no streaking.

## (2) Good (B):

Water beads on the paper. When the paper is shaken off the beads that remain may be slightly larger than the excellent and you may also get some slight streaking of the water. Over a 20 second period you may see some cockle to the paper where water has just started to penetrate the sheet. You must be able to write on the sheet with a ballpoint pen or a pencil with minimal to no streaking.

## (3) Poor (C):

Water does not bead and when the water is poured off the sheet it leaves behind evident streaks. Over a 20 second period you may see some increased cockle and water penetration into the paper.

The results are set forth in the figures and the following Table II.

TABLE II

| Substrate | 2 minute Cobb Felt Side Test, Felt Side | 2 minute Cobb Size Test, Wire Side | Felt Side Contact Angle | Wire Side Contact Angle | 'Watershedability' |
|-----------|-----------------------------------------|------------------------------------|-------------------------|-------------------------|--------------------|
| 1         | 37.7                                    | 39.9                               | 114.4                   | 98.6                    | C                  |
| 2         | 32.1                                    | 33.5                               | 128.1                   | 111.7                   | C                  |
| 3         | 26.0                                    | 29.5                               | 128.9                   | 126.4                   | C                  |
| 4         | 23.6                                    | 24.1                               | 130.2                   | 131.4                   | B                  |
| 5         | 21.9                                    | 23.1                               | 132.2                   | 131.3                   | A                  |
| 6         | 19.5                                    | 22.9                               | 133.0                   | 132.1                   | A                  |
| 7         | 23.5                                    | 22.6                               | 133.0                   | 133.9                   | A                  |
| 8         | 33.3                                    | 35                                 | 114.6                   | 101.2                   | C                  |
| 9         | 23.0                                    | 24.2                               | 131.7                   | 129.8                   | C                  |
| 10        | 20.6                                    | 21.6                               | 134.5                   | 134.2                   | B                  |
| 11        | 23.0                                    | 24.2                               | 135.0                   | 133.4                   | A                  |
| 12        | 21.1                                    | 21.1                               | 133.5                   | 134.5                   | A                  |
| 13        | 17.9                                    | 20.2                               | 131.9                   | 136.1                   | A                  |

## EXAMPLE III

Using the procedures of Examples I additional substrates were prepared. Process and product conditions are set forth in the following Table III.

TABLE III

| Substrate No. | Internal Sizing lb/Ton | Starch | Starch:\ Additive Wt Ratio | S.P. Solids | Pickup lb/Tons | Additives                                | Additive Pickup, % by wt Web | <sup>(3)</sup> Expandable Microspheres wt % |
|---------------|------------------------|--------|----------------------------|-------------|----------------|------------------------------------------|------------------------------|---------------------------------------------|
| 1             | 1.5                    | Yes    | 1:0                        | 8           | 37             | No                                       | 0.00%                        | 0                                           |
| 1B            | 1.5                    | Yes    | 1:0                        | 12          | 62             | No                                       | 0.00%                        | 0                                           |
| 2             | 3                      | Yes    | 1:0                        | 12          | 64.4           | No                                       | 0.00%                        | 0                                           |
| 3             | 4.5                    | Yes    | 1:0                        | 12          | 50.8           | No                                       | 0.00%                        | 0                                           |
| 4             | 4.5                    | Yes    | 2.3:1                      | 8           | 32             | <sup>(8)</sup> Additive 1                | 0.48%                        | 0                                           |
| 4B            | 4.5                    | Yes    | 2:1                        | 8           | 33.7           | <sup>(8)</sup> Additive 1                | 0.56%                        | 0                                           |
| 4C            | 4.5                    | Yes    | 1:1                        | 8           | 34.3           | <sup>(8)</sup> Additive 1                | 0.86%                        | 0                                           |
| 5             | 4.5                    | Yes    | 2:1                        | 8           | 32.4           | <sup>(7)</sup> Additive 2                | 0.53%                        | 0                                           |
| 5B            | 4.5                    | Yes    | 1:1                        | 8           | 35.2           | <sup>(4)</sup> Additive 3                | 0.88%                        | 0                                           |
| 6             | 4.5                    | Yes    | 2:1                        | 8           | 31.1           | <sup>(4)</sup> Additive 3                | 0.51%                        | 0                                           |
| 6B            | 4.5                    | Yes    | 1:1                        | 8           | 31             | <sup>(4)</sup> Additive 3                | 0.78%                        | 0                                           |
| 9             | 4.5                    | Yes    | 2:1                        | 8           | 33.8           | <sup>(5)</sup> Additive 5                | 0.56%                        | 0                                           |
| 9B            | 4.5                    | Yes    | 1:1                        | 8           | 33.3           | <sup>(5)</sup> Additive 5                | 0.83%                        | 0                                           |
| 10            | 4.5                    | No     | 0:1                        | 6           | 9.3            | <sup>(1)</sup> Additive 4, 6% Solids -   | 0.47%                        | 0                                           |
| 10B           | 4.5                    | No     | 0:1                        | 6           | 12.4           | <sup>(1)</sup> Additive 4, 4.6% Solids - | 0.62%                        | 0                                           |
| 11            | 4.5                    | Yes    | 2:1                        | 8           | 31.3           | <sup>(1)</sup> Additive 4                | 0.52%                        | 0                                           |
| 11B           | 4.5                    | Yes    | 1:1                        | 8           | 33.7           | <sup>(1)</sup> Additive 4                | 0.84%                        | 0                                           |

TABLE III-continued

| Substrate No. | Internal Sizing lb/Ton | Starch <sup>\</sup> | Starch: Additive Wt Ratio | S.P. Solids | Pickup lb/Tons | Additive Additives         | Additive Pickup, % by wt | ( <sup>3</sup> )Expandable Microspheres wt % |
|---------------|------------------------|---------------------|---------------------------|-------------|----------------|----------------------------|--------------------------|----------------------------------------------|
| 12            | 4.5                    | Yes                 | 10:1                      | 8           | 31.2           | ( <sup>9</sup> )Additive 9 | 0.14%                    | 0                                            |
| 12B           | 4.5                    | Yes                 | 1:1                       | 8           | 31.8           | ( <sup>9</sup> )Additive 9 | 0.80%                    | 0                                            |
| 12C           | 4.5                    | Yes                 | 10:1                      | 8           | 31.5           | ( <sup>6</sup> )Additive 6 | 0.14%                    | 0                                            |
| 13            | 4.5                    | Yes                 | 2:1                       | 8           | 29.5           | ( <sup>1</sup> )Additive 4 | 0.49%                    | 0                                            |
| 13B           | 1.5                    | Yes                 | 2:1                       | 8           | 35             | ( <sup>1</sup> )Additive 4 | 0.58%                    | 0                                            |
| 13C           | 1.5                    | Yes                 | 1:1                       | 8           | 34.6           | ( <sup>1</sup> )Additive 4 | 0.87%                    | 0                                            |
| 14            | 1.5                    | Yes                 | 1:1                       | 8           | 36.6           | ( <sup>5</sup> )Additive 5 | 0.92%                    | 0                                            |
| 15            | 1.5                    | Yes                 | 1:1                       | 8           | 36.5           | ( <sup>4</sup> )Additive 3 | 0.91%                    | 0                                            |
| 16            | 1.5                    | Yes                 | 1:1                       | 8           | 42.2           | ( <sup>1</sup> )Additive 4 | 1.06%                    | 2                                            |
| 16B           | 1.5                    | Yes                 | 1:1                       | 8           | 36             | ( <sup>1</sup> )Additive 4 | 0.90%                    | 2.5                                          |
| 17            | 1.5                    | Yes                 | 1:1                       | 8           | 41.2           | ( <sup>5</sup> )Additive 5 | 1.03%                    | 2                                            |
| 17B           | 1.5                    | Yes                 | 1:1                       | 8           | 40             | ( <sup>5</sup> )Additive 5 | 1.00%                    | 2.5                                          |
| 18            | 1.5                    | Yes                 | 1:1                       | 8           | 40.9           | ( <sup>4</sup> )Additive 3 | 1.02%                    | 2                                            |
| 18B           | 1.5                    | Yes                 | 1:1                       | 8           | 39.4           | ( <sup>4</sup> )Additive 3 | 0.99%                    | 2.5                                          |

The terms identified by superscripts are defined as follows:

(<sup>1</sup>)“Additive 4” is a stearylated melamine/paraffin wax based aqueous composition obtained commercially from RohmNova under the tradename Sequapel ® 414.

(<sup>2</sup>)“Starch” is an ethylated starch obtained commercially from Penford under the tradename Penford 270.

(<sup>3</sup>)“Microspheres” is a expandable microsphere obtained commercially from Expancel Inc. under the tradename “Expancel”.

(<sup>4</sup>)“Additive 3” is a styrene-butadiene copolymer based aqueous composition obtained commercially from Michelman under the tradename Vaportcoat 2200r.

(<sup>5</sup>)“Additive 5” is a poly(methylmethacrylate)/paraffin wax based aqueous composition obtained commercially from Spectra Kote under the tradename Spectra Guard 763 B.

(<sup>6</sup>)“Additive 6” is a styrene-acrylic acid copolymer based aqueous composition obtained commercially from Hercules under the tradename M 1322.

(<sup>7</sup>)“Additive 2” is a SBR (styrene-butadiene) based aqueous composition obtained commercially from Michelman under the tradename X300plus.

(<sup>8</sup>)“Additive 1” is an acrylic polymer based aqueous composition obtained from Progressive Coatings under the tradename Progressive J0819D.

(<sup>9</sup>)“Additive 9” is a styrene-maleic anhydride copolymer based aqueous composition obtained commercially from Hercules Incorporated under the tradename Scriptset 745.

## EXAMPLE IV

Using the procedures of Example II, the ability of the substrates of Example III to shed water was evaluated. The results are set forth in the following Table IV.

TABLE IV

| Expt No. | Cobb Size, Felt Side | Cobb Size, Wire Side | Watershedability |
|----------|----------------------|----------------------|------------------|
| 1        | 41.6                 | 43.5                 | C                |
| 1B       | 47.4                 | 49.3                 | C                |
| 2        | 46.9                 | 48.5                 | C                |
| 3        | 35.7                 | 33                   | C                |
| 4        | 30.8                 | 31.6                 | C                |
| 4B       | 29.9                 | 29.8                 | C                |
| 4C       | 30.8                 | 31.6                 | C                |
| 5        | 30                   | 26.8                 | C                |
| 5B       | 28.6                 | 29.1                 | C                |
| 6        | 27.7                 | 27.1                 | C                |
| 6B       | 23.4                 | 25.7                 | B                |
| 9        | 30                   | 30.1                 | C                |
| 9B       | 24.8                 | 24.9                 | B                |
| 10       | 25.2                 | 19.6                 | A                |
| 10B      | 22                   | 25.3                 | A                |
| 11       | 24.5                 | 22.8                 | A                |
| 11B      | 23.6                 | 21.4                 | A                |
| 12       | 31.7                 | 31.8                 | C                |
| 12B      | 31.7                 | 31.2                 | C                |
| 12C      | 31.6                 | 32.3                 | C                |
| 13       | 25.1                 | 26.7                 | B                |
| 13B      | 25.5                 | 25.8                 | A                |
| 13C      | 24.2                 | 25.1                 | A                |
| 14       | 26                   | 27.8                 | C                |
| 15       | 27.8                 | 32.7                 | B                |
| 16       | 18.4                 | 21.1                 | A                |
| 16B      | 18.5                 | 20.2                 | B                |

35

TABLE IV-continued

| Expt No. | Cobb Size, Felt Side | Cobb Size, Wire Side | Watershedability |
|----------|----------------------|----------------------|------------------|
| 17       | 24.1                 | 26.5                 | C                |
| 17B      | 17.7                 | 20.7                 | C                |
| 18       |                      |                      | B                |
| 18B      | 22.6                 | 23.2                 | B                |

40

What is claimed is:

1. A process of making a paper or paperboard, comprising contacting a paper or paperboard web at a size press with a composition comprising at least one hydrophobic polymer at an amount that is selected such that the paper or paper board exhibits a Cobb value that is equal to or less than 25 and exhibits a contact angle equal to or greater than 128°.
2. The process of claim 1 wherein the amount of said polymer is such that the Cobb Value is equal to or less than 23.
3. The process of claim 1, wherein the amount of said polymer is such that the Cobb Value is equal to or less than 20.
4. The process of claim 1, wherein the amount of said polymer is such that the paper or paperboard exhibits a contact angle equal to or greater than 130°.
5. The process of claim 1, wherein the amount of said polymer is such that the paper or paperboard exhibits a contact angle equal to or greater than 133°.
6. The process of claim 1, wherein the amount of said polymer is at least 0.4 wt % based on the dry weight of the paper or paperboard.

45

50

55

60

65

## 15

7. The process of claim 1, wherein the amount of said polymer is at least 0.5 wt % based on the dry weight of the paper or paperboard.

8. The process of claim 1, wherein the amount of said polymer is at least 0.9 wt % based on the dry weight of the paper or paperboard.

9. The process of claim 1, wherein the amount of said polymer is from 1.3 to 3.0 wt % based on the dry weight of the paper or paperboard.

10. The process of claim 1, wherein said composition comprises at least one sizing agent. 10

11. The process of claim 10, wherein said at least one sizing agent comprises starch.

12. The process of claim 11, wherein a weight ratio of starch to hydrophobic polymer picked up by the paper or paperboard web is less than 3 to 1. 15

13. The process of claim 11, wherein a weight ratio of starch to hydrophobic polymer picked up by the paper or paperboard web is less than 2 to 1.

14. The process of claim 11, wherein a weight ratio of starch to hydrophobic polymer picked up by the paper or paperboard web is less than 0.5 to 1. 20

15. The process of claim 1, wherein the hydrophobic polymer is selected from the group consisting of a styrene acrylic emulsion, styrene acrylic acid, styrene maleic anhydride, alkylated melamine wherein the alkyl moiety is branched or linear and has at least 7 carbon atoms, paraffin wax, polyurethane, hydrophobically modified starch, polyethylene, polymethylmethacrylate, alkyl ketene dimer, alkyl ketene dimer, and rosin. 25

16. The process of claim 1, wherein the hydrophobic polymer is selected from the group consisting of an alkylated melamine wherein the alkyl moiety is branched or linear and has at least 7 carbon atoms, and paraffin wax.

17. The process of claim 1, wherein the hydrophobic polymer is a combination of one or more alkylated melamines wherein the alkyl moiety is branched or linear and has at least 7 carbon atoms and one or more paraffin waxes.

18. The process of claim 1, wherein the hydrophobic polymer is a mixture of one or more alkylated melamine resins wherein the alkyl moiety is linear and has at least 13 carbon atoms and one or more paraffin waxes. 40

19. The process of claim 1, further comprising contacting the paper or paperboard web with at least one microsphere.

20. The process according to claim 1, comprising contacting the paper or paperboard web at a size press with a 45

## 16

composition comprising at least one sizing agent and at least one hydrophobic polymer at a weight ratio of sizing agent to hydrophobic polymer picked up by the paper or paperboard web that is less than 3 to 1; and wherein the paper or paper board exhibits a Cobb value that is equal to or less than 25.

21. The process according to claim 20, wherein the weight ratio of sizing agent to hydrophobic polymer picked up by the paper or paperboard web is less than 2 to 1.

22. The process according to claim 20, wherein the amount of said polymer is at least 0.4 wt % based on the dry weight of the paper or paperboard.

23. The process according to claim 20, comprising contacting the paper or paperboard web at a size press with a composition comprising starch and at least one hydrophobic polymer at a weight ratio of starch to hydrophobic polymer picked up by the paper or paperboard web that is less than 3 to 1; and wherein the paper or paperboard web comprises microspheres:

the paper or paper board exhibits a Cobb value that is equal to or less than 25; and

the paper or paper board exhibits a contact angle that equal to or greater than 128°.

24. The process according to claim 23, wherein the amount of said polymer is at least 0.4 wt % based on the dry weight of the paper or paperboard.

25. The process according to claim 1, wherein the at least one hydrophobic polymer is a plurality of hydrophobic polymers.

26. A process of making a paper or paperboard, comprising contacting a paper or paperboard web at a size press with a composition comprising at least one hydrophobic polymer and starch at an amount such that a weight ratio of starch to hydrophobic polymer picked up by the paper or paperboard web is less than 3 to 1, wherein the paper or paperboard exhibits a Cobb value that is equal to or less than 25. 35

27. The process according to claim 26, further comprising contacting the paper or paperboard web with at least one microsphere.

28. The process according to claim 26, wherein the paper or paperboard web comprises at least one microsphere.

29. The process according to claim 26, wherein the amount of said polymer is at least 0.4 wt % based on the dry weight of the paper or paperboard.

\* \* \* \* \*